

July 16, 1929.

E. R. ROSS

1,721,135

PROCESS OF CURING FRICTION MATERIAL

Filed March 12, 1927



Inventor

Elmer R. Ross

Hoover & Davis

Attorneys

## UNITED STATES PATENT OFFICE.

ELMER R. ROSS, OF BRIDGEPORT, CONNECTICUT, ASSIGNOR TO THE RAYBESTOS COMPANY, OF BRIDGEPORT, CONNECTICUT, A CORPORATION OF CONNECTICUT.

## PROCESS OF CURING FRICTION MATERIAL.

Application filed March 12, 1927. Serial No. 174,997.

This invention relates to a new and improved process of hardening a binder material in a fibrous stock, and more especially for the economical and efficient manufacture of friction materials having a fibrous base of asbestos or including asbestos, such for example as brake linings or clutch facings.

It is an object of the invention to produce a method for treating these materials, especially in curing or hardening the binder, which will give a better and a more uniform product than is now generally secured in the methods now employed, and also a method in which the time required for the curing operation is reduced over the methods now generally in use.

In the manufacture of friction materials or elements, and particularly friction materials having a woven asbestos yarn fabric base, it is customary to impregnate the fabric base with liquid binder substances, such as drying oils, asphaltic materials, pitches, heat setting synthetic resins and other adhesives or hardening substances, or substances catalyzing a hardening reaction, or solutions of the binders, and subsequently subject the impregnated fabric to air heat, such as in a furnace or oven, in order to harden the binder. For convenience I will call this method the "open curing method." In some binders a certain amount of oxidation is a desirable factor or may be an essential factor in the setting or hardening of the binder, such, for example, as the vegetable drying oils, but in the majority of other binders at present in use for friction materials the hardening of the primary saturant consists in the distillation or evaporation of the more volatile portions or the constituents having the higher vapor pressures at the curing temperatures, such as solvents contained therein, or some internal chemical change which induces hardening, or there may be a combination of both effects. This invention is especially advantageous for use in conditions where oxidation is a small, negligible or even an undesirable factor in the hardening of the binder, but it is also very advantageous for a preliminary or initial curing or treatment

in the hardening of certain binders where some oxidation is desired, as will be more fully discussed later.

As an example, it is known in the manufacture of brake linings to saturate tape made from a yarn consisting of asbestos fibre, cotton fibre and fine brass wire in a solution of gilsonite or other hard petroleum residue carried in a gas oil solvent, the latter selected for economy of price over other light solvents, such as benzol or gasoline. The saturated asbestos yarn tape is then heat treated in an oven in an oxidizing atmosphere having temperatures between about 350° F. and 450° F., whereupon the lower boiling gas oil distills away leaving the dry hard pitch as a residual binder. Depending on the temperature, the solvent used and the thickness of the stock, the time necessary for drying off the solvent may range from thirty minutes to several hours. It is noted that the higher the temperature and the shorter the time at that temperature in this open curing method the greater is the difference in hardness between the surface and the interior of the tape. This difference is due principally to the expansion of the saturant causing the excess to form a surface film and the more pronounced effect of oxidation, a surface phenomenon, at the higher temperatures. Above 450° F. this surface oxidation becomes so pronounced that spontaneous combustion frequently occurs, ruining the material. Also the cotton content of the fibrous base, which is a necessity in commercial asbestos yarn spinning and weaving, is very rapidly attacked by air heated above 350° F. decreasing the strength and pliability of the resultant brake lining. The case hardening of the film on the lining also reduces the pliability of the lining. Four serious disadvantages of air curing at elevated temperatures are, therefore, expansion of the saturant and its resultant gathering at the surface forming a film, case hardening of this film, rapid distillation and surface oxidation of this film which decreases the uniformity of curing of the fabric, and partial or complete destruction of the cotton fibre. Also, as

is well known, gases are very poor conductors and transmitters of heat, the heat conductivity of air, for example, being of the order of .000057 according to Winkelmann.

5 The present invention is designed to provide three factors which are extremely advantageous for rapid uniform curing and hardening of a binder material within a fibrous base, namely first, exclusion of air or 10 an oxidizing atmosphere, second, removal of excess saturant, and third, rapid conduction of heat to the material. Primarily the method comprises the immersion of the saturated fibrous mass, such as a brake lining, 15 within a heated liquid incompatible with the binder, or not affecting the hardening of the binder by chemical reaction. I use the term "incompatible" in the pharmaceutical sense as meaning not combining with or dissolving the binder. The distillation of the 20 more volatile components and/or internal heat setting of the binder thus take place with complete exclusion of air or an oxidizing atmosphere, and because of the fact that 25 liquids have a much greater thermal conductivity than gases, ranging from about ten times in organic liquids to about one hundred thousand times in molten metals, the required heat is much more rapidly supplied 30 to the article being treated and there is thus much more rapid penetration of the heat into the article. Thus for some purposes we have used a molten type metal alloy with a heat conductivity of about .11, which is 35 about twenty thousand times as great as that of air.

As a specific example we may saturate 40 brake lining tape made of asbestos covered wire yarn in a 30% solution of gilsonite in gas oil at 250° F. to complete saturation which may be about 40% of this saturant by weight. This may be led rapidly through a bath of type metal held at a temperature of 600° F. so that the total immersion time is 45 about three minutes. The saturant expands rapidly under the high temperature and about 20% of the saturant is released from the pores of the tape by this expansion and floats to the surface of the metal. The 50 residual saturant loses its gas oil solvent by distillation, the vapors also passing to the surface and out. The brake lining on exit from the bath is quickly cooled in an atmosphere of steam so as to prevent spontaneous combustion. After this treatment the gilsonite residue is left thoroughly distributed 55 in the brake lining in a substantially dry condition, and the brake lining after rolling to size is then ready for use.

60 It should be noted, as shown by the above example, that the present method allows the use of very much higher temperatures for distillation and curing than are safe for use where air or gases containing air is or are 65 the heat transferring medium, because of

the fact that the material under cure is sealed from the air. Under air or open curing temperatures for brake lining cures in excess of 450° F. are decidedly dangerous. The material can, therefore, with my improved method be exposed to much higher temperatures without burning. With this higher temperature and also the higher rate of heat transfer from the molten material, a much higher rate of distillation is possible 70 and no detrimental surface oxidation is produced. In the open process cure we cannot go above 450° F. safely without danger of burning, of course, depending on the material used, but this is with the materials 75 ordinarily used, while with the present method we can use as high temperatures as we please so long as it is not sufficiently high to produce detrimental carbonization of the materials, and of course, with the heated 80 liquid material in direct contact with the article being treated there is not only more rapid transfer of heat to the article but there is much more heat available at the surface 85 of the article.

90 The specific method above described is used merely as an example and this method is not necessarily limited to use with asbestos bases, but it may be used for any inorganic or noncombustible fibrous materials, or it 95 may be used with a combustible material with lower temperatures for the molten bath. Even with the use of combustible fibrous bases we secure a much improved product with a greatly reduced time required for the 100 curing or treatment because we may use higher temperatures than is possible with the open cure as the air is excluded, but the temperatures must be kept below the point at which the materials will carbonize to an 105 undesirable extent. The temperature of the metal bath should be sufficiently high so that droplets of the metal will not stick to the material treated.

110 In the accompanying drawing I have shown somewhat diagrammatically an apparatus which may be used in this treatment. In this drawing,

Fig. 1 is a vertical section through a furnace and saturating tank, and 115

Fig. 2 is a transverse vertical section showing a portion only of the furnace.

120 The furnace as shown comprises a chamber 5 in which the tank 6 is located carrying the molten metal or other heated liquid 7. Below the tank is a gas or oil burner 8 directed into a combustion chamber 9, and between the burner and the bottom of the tank are suitable baffles 10 and 11 of fire brick having 125 openings 12 and 13 respectively for passage of the products of combustion to the under side of the tank where they pass outwardly and upwardly at the outer sides of the tank through the flues 14 to the chamber 5. The tank is supported on suitable supports 130

At the opposite ends of the tank are guide drums 16 and 17 and between the drums are suitable rollers 18 mounted below the surface of the liquid to hold the tape 19 being 5 treated beneath the surface of the liquid. Above the drums 16 and 17 are guide drums 20 and 21 which are enclosed or separated from the chamber 5 by suitable walls 22. Outside the furnace is a tank 23 holding a 10 suitable saturant 24, the tank having suitable guide rollers 25 to hold the tape beneath the saturant. Scrapers 26 are provided at the outlet from the tank to scrape the surplus saturant from the tape as it leaves the tank. 15 At the outlet end of the tank 6 carrying the molten metal or other heated liquid used is a seal 27 of granular material, such as powdered charcoal carried by a swinging support 28. A block 29 composed of a pipe closed 20 at both ends secured to the lower end of this support will float in the metal and hold the support against the surface of the tape as it leaves the metal bath. A neutral or non-oxidizing atmosphere is maintained in the 25 chamber 30 where the tape is cooled after leaving the molten metal. This may be conveniently done by means of steam pipes 31 discharging into this chamber.

In operation the coil of the tape 32 is 30 mounted adjacent the saturating tank 23 and passes through the saturant in this tank, between the scrapers 26 and then through an opening 33 into the furnace where it passes over the drums 20 and 16 into the tank 6 35 where it passes through this tank under the molten metal or other heated liquid used. It then passes out the other end of this tank into the non-oxidizing atmosphere in the chamber 30 where it is rapidly cooled to a 40 temperature below the temperature which would cause spontaneous combustion if the tape were exposed to the air. It may then be wound up into a suitable coil, as shown at 34.

45 It will, of course, be understood that this is merely an example of how the process may be carried out and large variations in types of furnace may be used as found desirable. It will also be understood that a 50 number of different tapes may be passed through the furnace at the same time, as indicated in Fig. 2, and further that it is not necessary that the tape be saturated in a tank 23 associated with the heating furnace. In fact, it is sometimes desirable to 55 saturate the tape and then let it stand a certain time before heat treating. It will, of course, be understood that the time of immersion in the saturant and the time of immersion in the heated molten metal or other 60 liquid may be controlled by varying the sizes of the tanks and varying the rate at which the tape passes through the tanks.

65 It should be understood that the basic idea of this process of hardening binders in

fibrous or cellular materials is to heat the material within and by the medium of a heated liquid that does not interfere with the desired hardening, and it is capable of much variation and many uses that are not 70 described here. As has been shown, any binder material that depends for its hardening on the removal of its more volatile components, or on an internal chemical change resulting in hardening and which is induced 75 or accelerated by the application of heat, may be hardened within a molten metal. However, there are cases where molten metal may be undesirable and in these cases molten salts, for example, boric acid or 80 sodium sulphite, or waxes (paraffin, montan, etc.) fats, oils or other liquids may be used, the only requisite being that the liquid used for transmitting the heat shall not interfere with or prevent the desired hardening. 85 Molten metals are preferred as the heating medium because they do not wet or adhere to the article being heated. If hot oils or some material which does not combine with or dissolve the saturant but which adheres 90 to the article is used then, of course, a separate operation is required later to wash it off or dissolve it. For example, if we use as the binder a phenolic resin or a synthetic urea formaldehyde resin which is incompatible with paraffin or paraffin oil we effect the curing under this paraffin or paraffin oil and on the removal from the curing bath the layer of paraffin which adheres to the surface is dissolved off with gasoline 95 which does not affect the cured resin. During the heating in the paraffin the contained water will be evaporated and the hardening of the synthetic resin would take place by 100 polymerization. It will be apparent variations in the time of immersion as is found desirable may be regulated by the length of the dip, that is, the length of the path through the molten material, the speed of 105 movement of the material and the temperature of the bath.

110 It has been found that in open curing as above described there is a migration caused by expansion of the saturant which carries some of the binder out to the surface, so that in the open cure there is not a uniform distribution of the binder throughout the article at the end of the curing process, and there may be much less binder at the center 115 of the article as the greater proportion of it has been carried to the surface. This is partly due to the fact that in the open cure there is very slow transfer of heat to the interior of the article and most of the curing appears to be on the surface. In the present method the rapid heating causes the saturant to expand against the resistance of the liquid bath forcing the saturant uniformly and completely throughout the 120 fibres, also the more volatile constituents are 125

driven off within the article as well as at the surface, leaving the heavier or binding constituents substantially equally distributed throughout the fibre mass. This method, therefore, gives a more uniform product. In the specific example above given when asbestos covered wire was woven into a tape, the metal wire also assists in quickly transferring heat from the molten metal bath to the center and throughout the element being treated. This method can, therefore, be used as an initial curing to prevent subsequent migration of the binder to the surface where, as in certain types of binders or saturants, some oxidation is desired. With this type of binder the article is given a preliminary curing by this method to drive off the lighter constituents and remove excess of saturant which might later expand to the surface and form an undesirable film, and then it is given a cure in the open method to secure the oxidation desired. We can thus get a more uniform curing and a much more uniform final stock even though some oxidation is desired or some open curing is used. This method gives toughness without brittleness in the finished product.

In carrying out the method the melting point of the alloy should of course, be regulated according to the temperature desired for the curing. Metals with melting points from 350° F. to 625° F. or higher can be employed dependent upon the treatment being used, while with different materials temperatures may be used ranging from about 250° F. to a temperature which will not give undesirable carbonization of the stock used in the friction element, 250° F. being about the lowest temperature at which the curing can be effectively and practically carried out, although the curing is ordinarily carried out at a much higher temperature.

Having thus set forth the nature of my invention, what I claim is:

1. A process for making a friction element having an asbestos fibre base which includes treating the fibre with a primarily liquid binder, and then curing by heating the element within and by the medium of a liquid substantially incompatible with the binder at a temperature below that which would carbonize the base and sufficiently high to rapidly and uniformly cure and harden the binder.

2. A process for making a friction element which includes weaving a yarn having an asbestos fibre base into a tape, treating the tape with a normally liquid binder, and then curing by heating the tape within and by the medium of a liquid substantially incompatible with the binder at a temperature below that which would carbonize the yarn and sufficiently high to rapidly and uniformly cure and harden the binder.

3. A process for making a friction ele-

ment having an asbestos fibre base which includes treating the fibre with a primarily liquid binder and then curing by heating the element within and by the medium of a molten metal at a temperature below that which would carbonize the base and sufficiently high to rapidly and uniformly cure and harden the binder.

4. A process for making a friction element which includes weaving a yarn having an asbestos fibre base into a tape, treating the tape with a normally liquid binder, and then curing by heating the tape within and by the medium of a molten metal at a temperature below that which would carbonize the base and sufficiently high to rapidly and uniformly cure and harden the binder.

5. A process for making a friction element having an asbestos fibre base which includes treating the fibre with a primarily liquid binder and then curing by heating the element within and by the medium of a liquid substantially incompatible with the binder at a temperature below that which would carbonize the base and sufficiently high to rapidly and uniformly cure and harden the binder, and then exposing the element while heated to an oxidizing atmosphere to oxidize some of the binder at the surface of the element.

6. A process of making a friction element having an asbestos fibre base which includes treating the fibre with a primarily liquid binder, then removing the surplus binder by heating the element within and by a molten metal, and then exposing the element while heated to an oxidizing atmosphere.

7. A process of making a friction element having a fibre base which includes treating the fibre with a primarily liquid binder, then removing the surplus binder by heating the element within and by the medium of a liquid substantially incompatible with the binder, and then oxidizing some of the binder by exposing the element to an oxidizing atmosphere.

8. A process of making a friction element which includes weaving an asbestos covered wire into a tape, treating the tape with a normally liquid binder, and then curing this element by heating the element within and by a molten metal.

9. A process of making a friction element which includes weaving an asbestos covered wire into a tape, treating the tape with a normally liquid binder, removing the surplus binder by heating the element within and by the medium of a molten metal, and then curing in a heated oxidizing atmosphere.

10. The process of curing a friction element having a fibre base which includes treating the fibre with a hardening binder, then heating the element within and by the

medium of a molten metal, and then heating the element in contact with air to a sufficiently high temperature to oxidize some of the binder.

11. A process of making a friction element which includes weaving the element from asbestos covered wire, treating the ele-

ment with a normally liquid binder, and then curing by heating the element in and by the medium of a heated liquid substantially incompatible with the binder. 10

In testimony whereof I affix my signature.

ELMER R. ROSS.